

# United States Patent

[11] 3,523,541

[72] Inventor **Daniel Frishman**  
Andover, Massachusetts  
[21] Appl. No. **640,834**  
[22] Filed **May 24, 1967**  
[45] Patented **Aug. 11, 1970**  
[73] Assignee **Reid-Meredith, Inc.**  
Lawrence, Massachusetts  
a Corp. of Delaware

[56] **References Cited**  
UNITED STATES PATENTS  
1,845,752 2/1932 Johnson ..... 132/7  
2,692,182 10/1954 Nuessle ..... 8/115.5  
3,167,383 1/1965 Chezaud ..... 8/115.5

*Primary Examiner*— Robert Peshock  
*Assistant Examiner*— Gregory E. McNeill  
*Attorney*— Wilkinson, Mawhinney and Theibault

[54] **METHOD OF REMOVING FRIZZINESS FROM  
MODACRYLIC FILAMENTS AND IMPARTING  
CURL THERETO**  
13 Claims, No Drawings

[52] U.S. Cl. .... 132/5  
[51] Int. Cl. .... A41g 5/00  
[50] **Field of Search**..... 132/5, 7,  
38, 43.1, 53; 8/115.5, 116, 114.6; 167/Inquiry

**ABSTRACT:** The present invention relates to a method of straightening crimped, bent, kinked or otherwise non-straight modacrylic filaments used particularly in the synthetic hair styling art in pieces known as wigs, wiglettes, chignons and falls which is accomplished by immersing the stytable modacrylic filament in a heated solution of non-aqueous liquid, by way of example, of glycol or in an aqueous solution of saturated salt solution (sodium chloride) for 10-60 seconds at 160°-210°F.

**METHOD OF REMOVING FRIZZINESS FROM  
MODACRYLIC FILAMENTS AND IMPARTING CURL  
THERETO**

The present invention relates to method of removing frizziness from modacrylic filaments, particularly those filaments designated as stylable filaments extending from the artificial hairpiece described in my U. S. Letters Patent No. 3,139,093 granted June 30, 1964, which is manufactured in accordance with the process of my U. S. Letters Patent No. 3,199,516 granted August 10, 1965. The stylable filaments which extend from the base member of the artificial hairpiece and which are to be styled in various forms of hair-do's have presented problems of frizziness in the past. Frizz in a filament is a wave or crimp on almost a macroscopic basis which imparts tactile roughness and poor appearance. This is difficult to describe but the lack of smoothness results in a "glazed" artificial appearance.

Frizziness of modacrylic filaments has been a problem for a long time and can be caused during any one of several stages in the processing of the fiber and during manufacturing of the wig. During dyeing, particularly in a kettle, the fibers tend to contract, deform and to be shaped by their contact with adjacent fibers. These irregularities must be removed in order to have a smooth hair-like filament. Drying under tension can make the fiber smooth. On the other hand, the heat used during drying can also cause irregularities. A small amount of frizz can be imparted during preparation of the sliver. If curling temperature is too high or if the operator does not wind the hair on the roller tightly enough, frizzing results.

I have found it very difficult to strike a happy medium between imparting sufficient curl strength so that the curl stays in during washing and at the same time keeping frizz to a minimum. For example, if I increase the temperature during curling by 5° - 10°F. or increase the time by 10 - 15 minutes (195° - 225°F. for 45 - 75 minutes now being employed), increased frizziness results.

Dynel is a thermoplastic material which because of its largely amorphous nature has no clearly defined melting point. Instead it begins to soften as the temperature is increased and at the same time the fiber begins to contract (shrinks). The rate of these processes are dependent on the temperature, i.e., as the temperature is increased the tendency to soften and shrink goes up rapidly. Of course, Dynel would not be a practical textile material if these processes occurred at room temperature, but actually they begin to happen, although very slowly, even at temperatures as low as 150°F.

Thus, the heat somewhat softens the fiber and begins to make it contract slightly and if the fiber is put onto a roll or held in some other form during the time of heating and then cooled while in this configuration, a fairly permanent shape will be imparted. On a molecular basis what probably happens is that the increase in temperature breaks some of the weak secondary forces between the long chain molecules so that they can slide past each other (or uncoil) and then when they cool down new secondary forces form between the chain and the fiber stays in this new condition. Until it is heated again to a temperature at least as high as that which was originally used to set the fiber, it will maintain its new conformation. Severe mechanical manipulation causes changes in the fiber by actual fracturing of sections, etc., which can cause the fiber to lose some of its set.

The heat that is applied can be in the form of dry heat or steam heat or the fiber can actually be immersed in hot liquids. Indeed, some curling can be obtained by immersing the fiber in hot water but when one immerses modacrylic fibers in hot water another reaction begins to take place which commences above about 170°F. At this point, the fiber begins to swell and "vacuoles" or microscopic voids filled with water are formed. When this fiber is removed from the hot water and air-dried, these "vacuoles" do not collapse and instead a fiber which is full of little tiny air spaces which act as a delusterant results.

The tendency to deluster in water above about 170°F. is a problem when dyeing Dynel and Union Carbide carefully

recommends drying it at temperatures above 250°F. in order to reluster the fiber, or alternatively, suggests dyeing methods below 180°F. which results in only a small loss in luster.

In my work to remove frizz I observed that immersion of frizzy fibers in saturated salt solutions at elevated temperatures resulted in a spontaneous (without any external force applied) disappearance of frizz at temperatures in the range of 160° - 190°F., depending on the history of the specific dye lot. This procedure was found adaptable for use on fabric from which wigs are made or on the wigs themselves. However, since high temperatures are in themselves capable of setting a configuration, I found it necessary to brush the fabric and to orient the fibers into a straightened condition (on a macroscopic basis) before immersion into the hot saline. Also in order to keep the fibers straight it was helpful to brush the filaments while still warm, on their removal from the hot saline.

Similar results were obtained with hot non-aqueous liquids with the additional advantage that if the viscosity of the liquid is relatively high the fibers maintain their aligned and straightened orientation so that it is only necessary to brush before immersion.

We have explored the broad application of this principle which involves the use of liquids which do not swell Dynel. For the purpose of processing efficiency and cost it is desirable to use materials which are relatively inexpensive and which are easily washed off the filaments with water. Of the non-aqueous materials evaluation we have found the glycols to be most satisfactory. For example, Union Carbide's products Ucon H15N or H2N which are complex glycols are satisfactory for plant production. Ethylene glycol is satisfactory except that in some cases there results some bleeding of dyes.

All the frizz, bends, crimp, etc., when removed somehow "relaxed" the fiber so that in the subsequent curling operation there is little or no tendency to frizz when the curl was being set either with dry heat or by immersion in heated liquids.

I am not exactly sure of the mechanism of this pre-finishing or pre-conditioning treatment and why it then permits us to get better results. The fiber does not contract during this operation, in fact, some measurements made on individual fibers indicate that if anything, it elongates very slightly (1-2%). Furthermore, individual fiber work has shown that there is a very critical temperature at which this happens and this varies slightly from lot to lot, probably depending on the temperature used during dyeing, etc.

The spontaneous disappearance of frizz and the removal of the major bends give a very smooth fiber. Having this good base to work with and then curling properly achieves better results than I have ever had and what is most important less frizzing results during subsequent setting of the curl with heat. Perhaps the relatively simple explanation that the fiber is much straighter during actual curling so that it can be wound on the roller tighter is the most important factor.

Another important use for this technique of imparting curl with heated liquid is for "localized" curling. For example, in chignons or falls in which the Dynel fibers are about 16 inches long -- but only about 4 inches is desired to be curled at the end. I wrap the 4 inch end around metal rollers and then immerse the rollers into the heated liquid but I do not immerse the hair above the rollers. If dry heat is used and the whole fall is put into the oven, that portion above the 4 inch wrapped around the roller gets frizzy.

While the word modacrylic filament is used in the claims, it will be understood that this may be a single filament, a tow length of filaments or a fabric into which the filaments have been knit and extend from one side thereof for subsequent styling.

While the term brushing the filaments is employed in the claims, it will be appreciated that either brushing or combing are equivalents as long as it is a vigorous lineal action which tends to straighten the filament.

Although I have disclosed herein the best forms of the invention known to me at this time, I reserve the right to all such modifications and changes as may come within the scope of the following claims.

I claim:

1. The method of removing frizz from modacrylic filaments employed in articles such as wigs, fabrics, wiglets and other hairpieces to impart a straight natural hair-like appearance comprising:

- (a) immersing the article in a non-aqueous glycol liquid at an elevated temperature for a short time period.
- (b) removing the article from the liquid and allowing it to cool, and
- (c) rinsing the article to remove the liquid.

2. The method of Claim 1 wherein the temperature of the glycol is of the order of 200°F.

3. The method as claimed in Claim 2 wherein the period of immersion is of the order of 15 seconds.

4. The method of removing frizz from modacrylic filaments employed in articles such as wigs, fabrics, wiglets and other hairpieces to impart a straight natural hair-like appearance comprising:

- (a) immersing the article in a saturated solution of a salt of the group of sodium chloride, sodium sulfate, at an elevated temperature for a short time period.
- (b) removing the article from the liquid and allowing it to cool, and
- (c) rinsing the article to remove the liquid.

5. The method of Claim 4 wherein the temperature of the liquid is of a range of the order of 160° - 210°F.

6. The method of Claim 5 wherein the immersion is in multiple steps of 15 seconds duration each.

7. The method of straightening modacrylic filaments employed in articles such as wigs, fabrics, wiglettes and other hairpieces to remove frizz and to impart a straight natural hair-like appearance comprising:

- (a) immersing the article in a glycol at a temperature of the order of 200°F. for a period of 10-60 seconds,

35

(b) hanging the article and permitting the heated glycol to run off by gravity drain, and

(c) washing the article to remove the glycol.

8. The method of imparting curl to modacrylic filaments employed in articles such as wigs, fabrics, wiglets and other hairpieces comprising:

- (a) arranging the filaments into curls or rolls,
- (b) immersing the curled and rolled article into a non-aqueous glycol liquid at an elevated temperature for a short time period,
- (c) removing the article from the liquid and allowing it to cool, and
- (d) rinsing the article to remove the liquid.

9. The method of Claim 8, wherein the temperature of the glycol is of the order of 200 degrees Fahrenheit.

10. The method of Claim 9, wherein the period of immersion is of the order of fifteen seconds.

11. The method of imparting curl to modacrylic filaments employed in articles such as wigs, fabrics, wiglets and other hairpieces comprising:

- (a) arranging the filaments into curls or rolls,
- (b) immersing the curled and rolled article into a saturated solution of salt of the group of sodium chloride and sodium sulfate at an elevated temperature for a short time period,
- (c) removing the article from the liquid and allowing it to cool, and
- (d) rinsing the article to remove the liquid.

12. The method of Claim 11, wherein the temperature of the liquid is of a range of the order of 160 degrees to 210 degrees Fahrenheit.

13. The method of Claim 12, wherein the immersion is in a time period of the range of fifteen to sixty seconds.

35

40

45

50

55

60

65

70

75